

# UNITED STATES PATENT OFFICE.

OTTO SCHMIDT AND JULIUS MÜLLER, OF LUDWIGSHAFEN-ON-THE-RHINE, GERMANY,  
ASSIGNORS TO BADISCHE ANILIN & SODA FABRIK, OF LUDWIGSHAFEN-ON-THE-  
RHINE, GERMANY, A CORPORATION.

## TANNING MATERIAL.

1,089,797.

Specification of Letters Patent. Patented Mar. 10, 1914.

No Drawing.

Application filed January 21, 1913. Serial No. 743,297.

To all whom it may concern:

Be it known that we, OTTO SCHMIDT and JULIUS MÜLLER, subjects, respectively, of the King of Prussia and the King of Bavaria, residing at Ludwigshafen - on - the - Rhine, Germany, have invented new and useful Improvements in Tanning Materials, of which the following is a specification.

In the "Annalen der Chemie" (vol. 178, 10 1875, pp. 171 *et seq.*) Schiff has described the production of condensation products from phenol-sulfonic acid by heating it either with a large excess of phosphorus oxychlorid at from 50° to 60° C., or by 15 itself at about 200° C. at ordinary pressure, and states that the products are solid, and insoluble in dilute acids, and that, when used as tanning agents, they convert skins into a brittle leather. The leather obtained 20 is practically worthless and consequently the compounds described by Schiff have not been used commercially for tanning.

We have now found that by heating a phenol-sulfonic acid under mild conditions 25 we can obtain products which, in contradistinction to those described by Schiff, are eminently adapted for use as tanning agents especially in the manufacture of leather. Under the term "a phenol-sulfonic acid" 0 we include the sulfonic acids of phenol and of homologues thereof, particularly the cre- 5 sols. During the production of the new compounds, water is split off and condensation takes place, and we prefer, especially in the case of using phenol-sulfonic acid, to carry out the condensation under diminished pressure. If desired, a condensation agent (such for instance as phosphorus trichlorid, phosphorus oxychlorid, or thionyl chlorid) can be added, during the reaction, or, if desired, the products obtained by condensation without the addition of such an agent can be subsequently treated therewith. When employing phenol-sulfonic acids, no excess of the condensation agent should be em- 10 ployed, since otherwise products may be obtained which, like Schiff's aforesaid prod-

ucts, are not suitable for tanning purposes. When working with phenol-sulfonic acids at ordinary pressure, the temperature should 50 not exceed about 150° C. for any length of time. When producing tanning agents from cresol sulfonic acids, the conditions obtaining need not always be so mild as is desirable in the case of phenol sulfonic acids. 55

The products obtained according to this invention are probably bodies which are less highly molecular than those obtainable according to the method described by Schiff, and, when employed for tanning skins or 60 hides, full white leather of great softness and pliability can be obtained. As a general rule, the products of this invention are thick non-crystallizable syrups, but some approach a solid state on being cooled and 65 a few of those obtained from cresol sulfonic acids can be obtained in the solid state. Their alkali salts are colorless, amorphous and readily soluble in water, yielding intense colorations with ferric chlorid and 70 iron alum and, after the addition of acid, coagulate gum solution. The free acids are also generally soluble in dilute acids. Either the free acid or the alkali salt, in the presence of acid, is suitable for tanning skins or 75 hides, and they can be used, if desired, in admixture or conjunction with other tanning agents. Our new tanning agents contain sulfur and are also practically free from di- 80 phenylmethane compounds; consequently, on treatment in cold aqueous and slightly alka- line solution with a small quantity of alco- holic tetrachlorquinone, no coloring matter is formed.

The following examples will serve to illus- 85 trate further the nature of this invention, which, however, is not confined to these ex- amples. The parts are by weight.

Example 1: Heat phenol - para - sulfonic acid at a pressure of 20 mm. and at a tem- 90 perature of 130° C., for about 24 hours, or take test portions from time to time, dissolve them in water and add gum solution. When the precipitation which then occurs no

longer increases in quantity, the reaction is finished. The reaction product can be directly employed for tanning, or it can be purified by dissolving it in water, neutralizing with caustic soda solution, filtering and evaporating the filtrate to dryness, whereupon a white powder is obtained which rapidly dissolves and gives a clear solution in water. By ferric chlorid, the aqueous solution is colored red-violet. After acidification, it gives a considerable precipitate with gum solution. Skins or hides which have been tanned with a solution of the acid, or the acidified salt, are colored orange by iron alum.

Example 2: Heat, for 72 hours, at a pressure of 20 mm. and at a temperature of 140° C., the product obtained by heating phenol gently with concentrated sulfuric acid, which consists principally of phenol-para-sulfonic acid together with some phenol-ortho-sulfonic acid. Work up the reaction product as described in the foregoing example.

Example 3: Heat ortho-cresol-sulfonic acid (obtainable by sulfonating orthocresol in the cold, see *Berichte* 20, 3210) at a pressure of 20 mm. and a temperature of 130° C., for about 24 hours, or until a test portion, on being dissolved in water and on the addition of gum solution, shows that no further increase in the precipitation takes place. Then take up the product with water, filter, neutralize the filtrate with caustic soda and evaporate to dryness. The product is readily soluble in water and the solution is colored red-violet by ferric chlorid. After acidification, it yields a considerable precipitation with gum solution. By heating the product with dilute sulfuric acid, cresol is split off.

Example 4: Heat 1,000 parts of crude cresol-sulfonic acid at a pressure of about 20 mm. and at a temperature of 130° C., for about 24 hours, until a test portion shows that the reaction is complete. Then cool to about 80° C., add 186 parts of phosphorus trichlorid and stir for 1 hour at this temperature and at ordinary pressure. Then take up the product with ice and water, allow it to stand for some time and work up as described in the foregoing Example 3. The product is similar to that obtained according to the said Example 3.

Example 5: Heat together 3 parts of crude cresol-sulfonic acid and 1 part of para-phenol-sulfonic acid for 48 hours *in vacuo*, at a temperature of 133° C. When the mixture is cold, dissolve it in 18 parts of water, allow the solution to stand for some hours, filter it and then nearly neutralize the filtrate, so that about 5% of acid remains unneutralized. Cool in ice for 2 hours, filter

and evaporate to dryness. The product thus obtained is a light brown mass which rapidly dissolves in water and gives a copious precipitation with gum solution.

Example 6: Heat 225 parts of the sulfonation product of crude cresol with 262.5 parts of phosphorus oxychlorid for 4 hours at 60° C. Then distil off the excess of phosphorus oxychlorid, and wash the product with hydrochloric acid.

Example 7: Dissolve, in water, the product obtained according to the foregoing Example 3 and, if necessary, acidify it slightly, but not to such an extent that the skins or hides swell too much. The solution should have a density of about 0.6° Bé. Then hang the well-limed and bated skins or hides in the solution and gradually increase the quantity of tanning material and acid until, at the end of 10 days, the solution has a density of about 5° Bé. The process of tanning requires about 14 days. The leather is then neutralized and treated with fat and dried, which may be done in the usual manner. The leather is of excellent quality and does not become brittle on drying.

Either but one tanning bath can be employed or a series of two, three, or more such baths of different strengths can be employed, so that the skins or hides are subjected to the successive action of stronger tanning solutions.

Instead of employing the hanging process, the skins or hides can be tanned in other manner, for example according to the padding process, or in a drum, and in these cases the tanning liquid is preferably employed, from the start, in a more concentrated form, for instance from 2° to 4° Bé, and is subsequently also gradually strengthened. In this way complete tanning can be effected in from 6 to 8 hours, according to the material being tanned. In a similar manner, the tanning materials obtained according to others of the foregoing examples can be used for tanning.

Now what we claim is:—

1. As new articles of manufacture condensation products obtainable from a phenol-sulfonic acid, which new compounds contain sulfur, are practically free from diphenylmethane compounds, and in the form of their alkali salts are practically colorless, amorphous and readily soluble in water, yielding solutions which give intense colorations with ferric chlorid and, after the addition of acid, coagulate gum solution, and which tan hides giving a useful leather.

2. As a new article of manufacture the condensation product obtainable from cresol-sulfonic acid, which product contains sulfur, is practically free from diphenylmethane compounds, on heating with dilute

sulfuric acid splits off cresol, and in the form of its alkali salts is practically colorless, amorphous and readily soluble in water yielding solutions which give intense colorations with ferric chlorid, and after the addition of acid coagulate gum solution, and which tan hides giving a useful leather.

In testimony whereof we have hereunto

set our hands in the presence of two subscribing witnesses.

OTTO SCHMIDT.  
JULIUS MÜLLER.

Witnesses:

JOSEPH HEIFFER,  
J. ALEC. LLOYD.